

J. GITSHAM,  
PROCESS FOR THE MANUFACTURE OF THE SULFATE, SULFITE, AND OXID DIRECTLY FROM THE  
SULFID OF LEAD.  
APPLICATION FILED MAR. 21, 1916.

1,201,955.

Patented Oct. 17, 1916.

3 SHEETS—SHEET 1.



Fig. 1.



Fig. 6.

Fig. 7.



Fig. 5.

Inventor

James Gitsham

by *James L. Morris*

Attorney

Witnesses

*J. J. Bowes*

*M. E. Medade*

J. GITSHAM.  
PROCESS FOR THE MANUFACTURE OF THE SULFATE, SULFITE, AND OXID DIRECTLY FROM THE  
SULFID OF LEAD.  
APPLICATION FILED MAR. 21, 1916.

1,201,955.

Patented Oct. 17, 1916.

3 SHEETS—SHEET 2.



Fig. 1.



Fig. 2.



Fig. 3.

Witnesses  
J. L. Morris  
W. E. McAdae.

Inventor  
James Gitsham  
by *James L. Morris*  
Attorney

J. GITSHAM.  
PROCESS FOR THE MANUFACTURE OF THE SULFATE, SULFITE, AND OXID DIRECTLY FROM THE  
SULFID OF LEAD.  
APPLICATION FILED MAR. 21, 1916.

1,201,955.

Patented Oct. 17, 1916.

3 SHEETS—SHEET 3.



Witnesses:  
C. Reginald Culligan  
C. F. Stesler

Inventor  
James Gitsham  
by James L. Morris, Attorney

# UNITED STATES PATENT OFFICE.

JAMES GITSHAM, OF LONDON, ENGLAND.

## PROCESS FOR THE MANUFACTURE OF THE SULFATE, SULFITE, AND OXID DIRECTLY FROM THE SULFID OF LEAD.

1,201,955.

Specification of Letters Patent.

Patented Oct. 17, 1916.

Application filed March 21, 1916. Serial No. 85,664.

To all whom it may concern:

Be it known that I, JAMES GITSHAM, a subject of the King of Great Britain, residing at London, England, have invented a new and useful Improvement in Processes for the Manufacture of the Sulfate, Sulfite, and Oxid Directly from the Sulfid of Lead, of which the following is a specification.

This invention relates to an improved process for the manufacture of the sulfate, sulfite and oxid directly from the sulfid of lead.

According to my invention, the sulfid, *e. g.* in the form of ore, is introduced in a subdivided state into an electric furnace, preferably one in which the heating is effected by means of an electric arc, and is therein directly volatilized at a temperature not less than 5000 degrees F. and the resultant volatilized sulfid is subjected while in a heated condition to the action of oxygen, the product of the reaction, which consists mainly of lead sulfate, lead sulfite and a trace of lead oxid, in the form of an impalpable powder, being then separated from the gaseous medium in which it is suspended. This powder is of a suitable consistency for mixing directly with a drying oil in order to form a paint.

Since the primary material is sulfid ore taken substantially in the form in which it is obtained from the mine and suitably reduced in size, and since the only reagent employed with such primary material is atmospheric air, no fluxes or the like being required, it will be seen that the process is an extremely economical and simple one. Moreover since the heat is generated by electrical means, the powdery product and consequently the paint prepared therefrom can be obtained of a very pure color. Such paint will consist almost entirely of compounds, *e. g.* lead sulfate and sulfite, of a non-poisonous nature, so that, assuming sulfid ores of a suitable degree of purity are available, a pure white pigment can be obtained containing only a very small proportion of poisonous matter, thus fulfilling the requirements of modern hygiene.

The oxidation of the volatilized sulfid may be advantageously effected by the oxygen of atmospheric air supplied to the volatilized material mainly after the latter has left the electric furnace but while it is still at an

elevated temperature. This may be effected by withdrawing the volatilized material from the electric furnace through an education flue or combustion chamber by means of a suitable exhausting device and then introducing air into said flue or chamber in order to oxidize the heated volatilized material therein.

In order to prevent clogging of the furnace, and also to assist in the starting in operation of the apparatus, a suitable amount of air is admitted to the furnace itself, this air serving as a carrier for the volatilized material and also supplying oxygen for initiating the oxidation of the sulfid into sulfate and sulfite of lead.

In each case the air supplied to the volatilized material may be advantageously pre-heated, *e. g.* by heat withdrawn from the air or other gases in the apparatus beyond the point where the oxidation of the volatilized material is complete.

The products of the oxidation are collected in an extended passage or passages provided with baffles and into which the volatilized and oxidized material is delivered by the device whereby it is exhausted from the electric furnace. The baffles near the outlet end of the collecting passage may be advantageously sprayed with oil to enable the last traces of powdery material to be removed from the gaseous medium (*e. g.* air from which a large proportion of the oxygen has been removed by the oxidation) in which this product is suspended. This oil may advantageously consist of linseed or other drying oil suitable for use in the preparation of a paint.

In the accompanying drawing I have shown how my said invention may be conveniently and advantageously carried into practice.

In this drawing, Figure 1 is a diagrammatic side elevation of the complete plant. Figs. 2 and 3 are vertical sections taken on planes at right angles to each other, and Fig. 4 is a horizontal section, showing the electric furnace drawn to a larger scale. Figs. 5 and 6 are respectively a horizontal and a vertical section showing the arrangement for spraying with oil the baffles in the depositing passage. Fig. 7 is a transverse section of the depositing passage illustrating a modification. Figs. 8 and 9 are, respec-

2

tively, a side and a front elevation of the exterior of the furnace showing details of construction.

The electric furnace A comprises an outer 5 casing of firebrick with an inner lining of magnesite bricks or other suitable fire-resistant material. Across the bottom of the furnace there extends a cast iron plate B, which is covered with carbon slabs C, C, so 10 as to form one electrode, *e. g.* the negative electrode of the furnace. The other electrode, the positive electrode, consists of a carbon rod D provided with suitable controlling mechanism, whereby an arc may be 15 maintained in the interior of the furnace A. For example, as shown in Figs. 8 and 9, the carbon rod D can be mounted in a holder 4 slidable in suitable guides 5, 5 and counterbalanced by a weight 6 connected to such 20 holder by a wire rope, chain or the like 7 extending over a pulley 8. The carbon rod can be fed forward into the furnace in any suitable manner, for example by means of a rack 9 on said holder engaging a pinion 10 25 actuated through a hand-wheel 11, the rate of feed being preferably such as to maintain the current at a constant value.

E is a suitable source of electric energy, here shown as a continuous current dynamo. 30 E' is the connection between the dynamo and the plate B.

In the upper wall of the furnace, there is arranged a feed hopper F, in the delivery chute of which an Archimedean screw G is 35 rotatably mounted and driven, *e. g.* through bevel and belt gearing H, J, so as to insure that the sulfid ore or other sulfid shall be fed to the arc at a uniform rate.

K is a tap-hole, through which the slag or 40 other residue that is not volatilized by the arc can be drawn off. When not in use, this tap-hole is closed by means of fire-clay.

M is an inlet controlled by a valve N for 45 enabling air to be supplied to the interior of the furnace, in order to oxidize the material volatilized by the arc. O is the outlet for the air, volatilized material and the products of the reaction between the oxygen of said air and the volatilized material. 50 This outlet communicates with a flue P which is also provided with an air-inlet Q controlled by a damper or valve R and is preferably formed of fire-brick or other suitable refractory material, so that its interior

55 is capable of being heated to a high temperature, *e. g.* at the part near the furnace, where the burning or oxidation of the sulfid into sulfate and sulfite mainly takes place. The products of the reaction are drawn along 60 the flue P by means of an exhausting fan S, whereby they are delivered into the inlet end of a depositing passage T provided with baffles U, U. The outlet end of the passage T is in communication with the bottom of 65 a chimney stack V, whereby the contents of

the flues P, T are carried along in the direction away from the furnace. In order to insure that the gases discharged into the atmosphere shall not carry with them any of the powdery products of the reaction, oil is 70 sprayed from the nozzles W, W on to the baffles U, U, the last traces of dust contained in the gases being caught in the oil and retained for use.

An advantageous length of the flue P has 75 been found to be about 150 feet, the air-inlet Q being arranged at from 8 to 25 feet from the furnace. An advantageous length of the depositing passage T is 600 feet. These dimensions are, however, only given by way of 80 example.

The air for oxidizing the volatilized materials can be heated on its way to the inlets M, Q by passing it through a conduit 1, which is formed of metal of good thermal 85 conductivity and is arranged in the passage T, see Fig. 7. This conduit is made with an inwardly turned portion 2, in order to subject all the air therein to the heat from the gases outside. Moreover its outer surfaces 90 are inclined as shown so as to prevent accumulation thereon of the powdery products of the reaction. Air-conduits of any other suitable shape may however be employed for 95 this purpose.

The operation is as follows:—When dealing with lead sulfid ore, it is fed in a suitable state of subdivision, for example crushed to a fine state, into the arc in the furnace, and air is admitted at one or both 100 of the inlets M, Q. The lead sulfid in the ore will thereby be immediately volatilized and subsequently oxidized by the oxygen of the air admitted, so as to form a mixture of sulfate, sulfite and oxid, the heat of combustion of the sulfur assisting in maintaining the temperature necessary for the reaction. The powdery material formed gradually deposits itself in the flue P and passage 105 T and is collected and removed therefrom in 110 any suitable known manner.

Since the powdery material obtained as above described is of a suitable consistency for the manufacture of paint, it can be readily converted into the same by grinding or 115 mixing with linseed oil or other suitable drying oil.

When starting operations, the major portion of the air is preferably admitted at the inlet M. When, however, the flue P has 120 been heated up to a temperature suitable for the oxidation of the volatilized material, the supply of air through the inlet Q can be increased and that through the inlet M decreased.

I claim:

1. A process of obtaining sulfate, sulfite and oxid directly from the sulfid of lead, said process consisting in introducing the sulfid in a subdivided state into an electric 130

furnace, directly volatilizing the same in such furnace, subjecting the resultant volatilized material while in a heated condition to the action of oxygen, and then separating the product of the reaction from the gaseous medium in which it is suspended.

2. A process of treating lead sulfid ore, consisting in volatilizing in an electric furnace the ore which has been suitably reduced

in size and oxidizing the volatilized material, thereby forming a mixture of lead sulfate, lead sulfite and lead oxid adapted for use as a color or pigment, substantially as described.

JAMES GITSHAM.

Witnesses:

GEORGE HARRISON,  
CONRAD K. FAL RENSTEIN.